

## UNITED STATES PATENT OFFICE

FREDERICK M. BECKET, OF NEW YORK, N. Y., ASSIGNOR TO ELECTRO METALLURGICAL COMPANY, A CORPORATION OF WEST VIRGINIA

## PROCESS OF MAKING LOW-CARBON CHROMIUM ALLOYS

No Drawing.

Application filed March 12, 1927. Serial No. 175,009.

This invention relates to the art of making low-carbon chromium alloys typified by rustless iron. The object of the invention is to provide a novel and economical process for 5 preparing such alloys.

Rustless iron for the purposes of this invention may be defined as an alloy consisting essentially of iron and chromium, with upward of about 9% of chromium and less 10 than 0.2% of carbon. Nickel may also be present in varying proportions replacing the iron. A preferred composition contains about 12%-14% of chromium with 0.12% or less of carbon. Another excellent composition 15 contains around 16%-18% of chromium, with 7%-8% nickel and carbon around 0.12% or less.

Such alloys have heretofore been made by various processes, such as the introduction 20 of low-carbon ferrochrome or chromium metal into a bath of low-carbon iron; or by subjecting an iron-chromium alloy containing more than the desired proportion of carbon to an oxidizing treatment to eliminate 25 a portion of the carbon, and thereafter de-oxidizing the resulting low-carbon product, as disclosed in United States Patent 1,365,091 to Clement.

In the process disclosed in the Clement patent, 30 the final step of deoxidizing the metal is necessary because of the oxygen which the bath takes up in the decarburizing stage. This oxygen content and the necessity for its removal are discussed in the patent on 35 page 3, beginning at line 100.

In an extensive experience with the Clement process I have confirmed the patentee as to the ability of his process to produce rustless alloys of good quality, and have in fact 40 demonstrated that the process is in all respects a meritorious one. I have nevertheless developed certain improvements in the process, and these improvements form the subject of the present application.

In the Clement process, deoxidation of 45 the metal is effected by means of a so-called "carbide" slag, prepared by removing the slag used in the preceding stage, covering the surface of the metal with lime and melting 50 down the latter at a very high temperature,

and then introducing powdered coal or coke. The slag thereupon acquires a reducing character, and when the metal has remained in contact with it for a sufficient time at high temperature, deoxidation of the metal is complete and the heat is ready for pouring. Since the decarburizing slag is removed from the furnace before the reducing agent is added, the chromium contained in this slag is completely lost. I have found that the deoxidation 5 can advantageously be carried out by means other than those described in the patent.

The use of a "carbide" slag as described in the patent necessitates very high temperatures and thorough agitation of the metal with the slag. These conditions favor the oxidation of chromium and the losses of the latter are apt to be rather high. In addition great care must be exercised in forming the slag to avoid re-carburizing the metal.

I prefer to deoxidize with a reducing agent which is non-carbonaceous, whereby all risk of re-carburizing the bath is avoided. In some cases the object is to diminish the carbon content of the metal to 0.05% or even less, and in view of the avidity with which chromium alloys take up carbon it is necessary to use every precaution to avoid introduction of carbon in the later stages of the process.

The deoxidizing agents which I employ act more rapidly than the carbonaceous materials described by Clement, and because of this more rapid deoxidation the time is diminished during which the heat is subjected to the carbon-bearing atmosphere of the furnace, this being an advantage of some importance where metal of a very low carbon content is the objective. I prefer to use silicon or its alloys as deoxidizers, for example ferrosilicon, or silicon alloys containing one or more of the elements chromium, manganese, magnesium, calcium, zirconium, aluminum or titanium, with or without considerable quantities of iron. The invention is not restricted to the use of silicon alloys, however, and other deoxidizers may be used. A plurality of deoxidizers sometimes gives the best

results. For example, an addition of one of the silicon alloys referred to above may be followed by an addition of aluminum or other extremely energetic deoxidizer.

5 The following specific example will further illustrate the process:

*Example I.*—Fourteen hundred twenty parts of low-carbon steel scrap, 150 parts of lime, and 50 parts of quartzite were melted 10 down together and 580 parts of high-carbon ferrochrome containing Cr 69.2%, C 4.79%, and Si 1.80% was then added, meanwhile keeping the bath fluid. This was followed by 100 parts of chrome ore added in three 15 portions, one hour intervening between additions. About an hour after the last addition of ore the carbon had fallen to 0.06% and the first slag was poured off.

A new slag was then formed, the ingredients and their quantities being the same as before. When this slag had become fluid, 60 parts of 50% ferrosilicon was added in four lots at intervals of 5 minutes. Shortly after the last addition 17 parts of low-carbon ferromanganese (Mn 82.5%, Si 1.03%, C 0.13%) was added and the heat tapped and poured into ingot molds. Only 35 minutes elapsed between the removal of the first slag and the tapping of the metal.

30 The finished metal contained Cr 12.13%, C 0.06%, Si 0.18% and Mn 0.35%. The metal poured well and all the ingots had good shrinkage.

The substitution of a metallic deoxidizing agent for a carbon-containing slag, as described above, permits a further modification of the Clement process under some conditions. This modification consists in the elimination of one of the slags, and it can be followed when the raw materials used in making the rustless iron are very low in phosphorus and sulphur. In the one-slag process the deoxidizer is introduced into the furnace at the end of the decarburization, without previously tapping the slag. Under these conditions there is a tendency for phosphorus and sulphur to pass from the slag to the metal, and the content of these elements in the slag at the end of the decarburizing stage must therefore be low. The one-slag process is especially applicable where an extremely low carbon content is not required, but it may be used even in this case under proper conditions. When the single-slag modification can be used 55 a considerably increased recovery of chromium can be achieved because chromium is returned to the metal from the decarburizing slag.

The following example illustrates the modification last described:

*Example II.*—Lime (200 parts) and quartzite (100 parts) were melted down in a basic-lined electric furnace, and 970 parts of high-grade low-carbon steel scrap and 280 parts 65 of high-carbon ferrochrome were then added.

The ferrochrome analyzed Cr 70.62%; C 6.51%; Si 1.15%. Forty parts of chrome ore was then added to the slag and the bath was maintained at high temperature until the carbon was slightly less than 0.10%. Forty-five parts of 12 mesh 95% ferrosilicon was 70 then scattered on the slag in successive small portions, 5 pounds of lime being also introduced for each pound of Si in the ferrosilicon thus added, thus maintaining the basicity of 75 the slag. When the metal was sufficiently deoxidized, a small amount of manganese was introduced by the addition of 10 parts of low-carbon ferromanganese, and 10 minutes later the heat was tapped. A small quantity 80 of silicon-zirconium was added to the ladle in accordance with established steel-making practice. The alloy analyzed Cr 13.17%; C 0.10%; Si 0.38%; Mn 0.54%. It will be 85 noted that in the foregoing example, the number of pounds of silicon introduced as ferrosilicon during the process is greater than the number of pounds of chrome ore charged to the furnace. Therefore the silicon added is largely in excess of that required 90 to reduce the oxides of chromium and iron contained in the ore. This results in a reduction of a high proportion of the chromium in the slag, greatly increasing the recovery of 95 chromium.

The procedure given in the Example II may be advantageously modified by adding a very energetic deoxidizer such as aluminum to the metal in the furnace after the action of the first deoxidizer (ferrosilicon) is substantially complete. The quantities of silica used in the specific examples for making up the slags tend to facilitate the manipulation of the furnace, but slags of a more basic character expedite deoxidation of the metal 100 and are preferable on that ground.

The term "high-carbon ferrochrome" as used in the specification and claims refers to a product characterized by a relatively high ratio of carbon content to chromium content, 105 and made by reducing a chromium-oxide-containing material with carbon under conditions permitting carburization of the reduced metal. Where the appended claims refer to combining high-carbon ferrochrome with iron 110 it will, of course, be understood that the materials may be combined either directly or indirectly, and in any one of a number of different ways, some of which are enumerated in the Clement Patent Number 1,365,091. 115

I claim:

1. The process of making iron-chromium alloys low in carbon which comprises combining high-carbon ferrochrome with low carbon iron to form a melt having a chromium content at least as high as that desired in the finished alloy; said melt containing an excess of carbon and being covered by a slag; adding chromite to said slag, maintaining the melt at a high temperature under the slag to 125 130

decarburize the metal, whereby the slag becomes rich in chromium; and then, without removing the slag, deoxidizing the metal and recovering a substantial proportion of chromium from the slag by adding silicon to the slag while keeping the latter in a basic condition.

2. The process of making rustless iron which comprises combining high-carbon ferrochrome with iron to form a melt in which the ratio of the carbon content to the chromium content is materially higher than in rustless iron, providing on said melt a covering slag containing an oxide of a metal of the group consisting of iron and chromium, maintaining the melt at a high temperature thereby oxidizing the excess carbon and incidentally a substantial part of the chromium in the melt, the chromium oxide thus formed passing into the slag, and then, without removing the slag, subjecting the slag to the action of a non-carbonaceous reducing agent whereby to reduce a substantial proportion of the chromium oxide content thereof.

25 3. The process of making rustless iron which comprises combining high-carbon ferrochrome with iron to form a melt in which the ratio of the carbon content to the chromium content is materially higher than in rustless iron, providing on said melt an oxidizing covering slag containing an oxide of a metal of the group consisting of iron and chromium, maintaining the melt at a high temperature thereby oxidizing the excess carbon and incidentally a substantial part of the chromium in the melt, the chromium oxide thus formed passing into the slag, and then, without removing the slag, subjecting the slag to the action of silicon whereby to reduce a substantial proportion of the chromium oxide content thereof.

4. The process of making rustless iron which comprises combining high-carbon ferrochrome with low-carbon iron to form a melt in which the ratio of the carbon content to the chromium content is materially higher than in rustless iron, providing on said melt a basic lime silica slag containing chromium oxide, maintaining the melt under said slag at a high temperature thereby oxidizing the excess carbon and incidentally a substantial part of the chromium in the melt, the chromium oxide thus formed passing into the slag, and then, without removing the slag, and while keeping it in a basic condition, subjecting the slag to the action of silicon to reduce a substantial proportion of the chromium oxide content thereof.

5. The process of making rustless iron which comprises combining high-carbon ferrochrome with low-carbon iron to form a melt in which the ratio of the carbon content to the chromium content is materially higher than in rustless iron, and in which the chromium content is at least as high as that de-

sired in the finished alloy, providing on said melt a slag containing chromium oxide, maintaining the melt under said slag at a high temperature thereby oxidizing the excess carbon and incidentally a substantial part of the chromium in the melt, the chromium oxide thus formed passing into the slag, and then, without removing the slag, and while keeping it in a basic condition, subjecting the slag to the action of a non-carbonaceous reducing agent whereby to reduce a substantial proportion of the chromium oxide content thereof.

6. The process of making rustless iron which comprises combining high-carbon ferrochrome with iron to form a melt in which the ratio of the carbon content to the chromium content is materially higher than in rustless iron, said melt being covered by a slag, adding chromite to said slag, maintaining the melt at a high temperature thereby oxidizing the excess carbon and incidentally a substantial part of the chromium in the melt, the chromium oxide thus formed passing into the slag, and then, without removing the slag, subjecting the slag to the action of a non-carbonaceous reducing agent whereby to reduce a substantial proportion of the chromium oxide content thereof.

7. The process of making rustless iron which comprises combining high-carbon ferrochrome with low-carbon iron to form a melt in which the ratio of the carbon content to the chromium content is materially higher than in rustless iron, and in which the chromium content is at least as high as that desired in the finished alloy, said melt being covered by a basic lime silica slag, adding chromite to said slag, maintaining the melt under said slag at a high temperature thereby oxidizing the excess carbon and incidentally a substantial part of the chromium in the melt, the chromium oxide thus formed passing into the slag, and then, without removing the slag, and while keeping it in a basic condition, subjecting the slag to the action of silicon to reduce a substantial proportion of the chromium oxide content thereof.

In testimony whereof, I affix my signature.

FREDERICK M. BECKET.

120

125

130